

## UNITED STATES PATENT OFFICE

2,397,332

## TRANSFORMER OILS

Earl Amott, Long Beach, Calif., assignor to Union  
Oil Company of California, Los Angeles, Calif.,  
a corporation of California

No Drawing. Application January 2, 1942,  
Serial No. 425,451

4 Claims. (Cl. 252—64)

This invention relates to mineral oils adapted for use as transformer oils and in connection with similar electrical equipment. The particular object of the invention is to produce a transformer oil having high resistance to oxidation even in the presence of copper.

Primarily the invention resides in a light mineral oil, such as is commonly used for electrical transformers, containing a very minor proportion in the order of a few tenths of one percent of a tartaric acid ester.

In practicing the invention, a considerable number of tartaric acid esters have been tested. These tests have included the tartaric acid esters of secondary alcohols and primary alcohols, including straight chain alcohols and branched chain and cyclic alcohols such as cyclo-hexyl and benzyl alcohols. The esters of the branched chain and cyclic alcohols constitute an important group especially the cyclo-hexyl, iso-propyl, iso-amyl and benzyl esters. Evidently, the cyclics may, for this purpose, be considered branched. Viewed from another standpoint, the esters of the secondary alcohols are very desirable, and perhaps preferable especially since the cyclo-hexyl and iso-propyl esters have proved so far to be respectively the best. The esters of the straight chain alcohols containing less than about ten carbon atoms are also quite desirable, especially the butyl esters. However, no tartaric acid esters have been tested which do not appear to be sufficiently valuable to have some importance.

The invention extends to these groupings as indicated. Preferred individuals are di-cyclo-hexyl tartrate, di-iso-propyl tartrate, di-butyl tartrate, di-iso-amyl tartrate and di-benzyl tartrate in the order indicated.

In preparing transformer oils in accordance with this invention, a usual light mineral oil employed in electric transformers and well known to the industry has about 0.2% of the selected tartrate dissolved therein. This particular amount does not appear to be critical inasmuch as smaller proportions such as 0.05% yield an appreciable anti-oxidant effect, and inasmuch as larger percentages afford equally good protection and possibly somewhat better protection in some instances, although it does not appear that any additional advantage is obtained when the percentage of ester is increased above about 0.5%.

The preparation of transformer oils according to this invention requires nothing more than the simple solution of the small percentage of the selected ester of tartaric acid in the oil.

Oils which have been made and tested containing specific esters are shown in the accompanying table. The first column of figures gives

sludge and acid number and indicates results of what has been considered a very severe test. Here the oil was heated in the presence of copper for seven days at the distinctly elevated temperature of 120° C. These oils which showed sludge and acid number of less than about 1.0 in this seven day test and did not show undue darkening, are considered especially valuable.

However, this test in the presence of copper eliminates a number of oils which will be adequate for commercial uses. For these purposes the less severe test shown in the second column of sludge and acid numbers was made on each oil. This test consisted of heating the same specimens at the same temperature of 120° C. for forty-five days in the absence of copper, as distinguished from heating in the presence of copper for the seven day test. In this less severe test, the esters of secondary butyl alcohol, the octyl alcohol, and the higher carbon content lauryl and stearyl alcohols, which gave sludge or acid numbers approximating 1.0 or more in the severe test, showed good results in the less severe test. This indicates these materials to be good at least for ordinary commercial purposes. Even the unsaturated allyl alcohol ester is adequate. It was difficult to obtain pure alcohols of the lauryl and stearyl types for test. It is likely that esters of the pure alcohols will rate higher.

Transformer oils heated at 120° centigrade in glass with indicated esters

|    | Oil containing 0.20% of tartaric di-ester of— | Copper present, heated 7 days |          | Copper absent, heated 45 days       |                |
|----|-----------------------------------------------|-------------------------------|----------|-------------------------------------|----------------|
|    |                                               | Sludge, ml./10 ml. oil        | Acid No. | Sludge, ml./10 ml.                  | Acid No.       |
| 35 | No additive—                                  | 1.08                          | 1.07     | 0.30.....                           | 0.96.          |
| 40 | Secondary alcohols:                           |                               |          |                                     |                |
|    | Cyclohexyl.....                               | 0.45                          | 0.66     | None.....                           | 0.28.          |
|    | Isopropyl.....                                | 0.70                          | 0.89     | do.....                             | 0.47.          |
|    | Sec. amy.....                                 | 0.83                          | 0.95     | Moderate improvement over base oil. |                |
|    | Sec. butyl.....                               | 1.33                          | 1.38     | None.....                           | Less than 0.5. |
| 45 | Primary alcohols:                             |                               |          |                                     |                |
|    | Branched chain or cyclic—                     |                               |          |                                     |                |
|    | Benzyl.....                                   | 0.31                          | 0.44     | Improvement over base oil.          |                |
|    | Isoamyl.....                                  | 0.65                          | 0.83     | None.....                           | 0.13.          |
|    | Isobutyl.....                                 | 0.77                          | 0.71     | Moderate improvement.               |                |
|    | 2-ethylhexyl (octyl).                         | 0.93                          | 0.87     | Improvement.                        |                |
| 50 | Straight chain—                               |                               |          |                                     |                |
|    | Butyl.....                                    | 0.65                          | 0.78     | None.....                           | 0.29.          |
|    | Methyl.....                                   | 0.75                          | 0.77     | do.....                             | Less than 0.5. |
|    | Ethyl.....                                    | 0.85                          | 0.88     | do.....                             | Less than 0.5. |
|    | Allyl.....                                    | 0.83                          | 0.95     | Improvement.                        |                |
|    | Lauryl.....                                   | 0.99                          | 1.02     | 0.4.....                            | 0.84.          |
| 55 | Stearyl.....                                  | 1.75                          | 1.48     | None.....                           | Less than 0.5. |

In the above table the sludge indication of milliliters of sludge per ten milliliters of oil is

for color conversion. The only ones that might be considered objectionably dark were the specimens containing the secondary butyl ester, the the standard ASTM precipitation number. Most of the materials tested produced at the most only very slight darkening in the oils in usual tests allyl ester, the stearyl ester and the octyl ester. But even these, at least upon the basis of the forty-five day test in the absence of copper, appear to possess value.

Applicant does not mean to be limited to the specific materials listed, because it is evident that other esters apparent to the skilled chemist will yield satisfactory results.

I claim:

1. A mineral transformer oil consisting essentially of a light mineral oil of the transformer oil

type and a small proportion, less than about 0.5%, sufficient to inhibit oxidation of said transformer oil, of a tartaric di-acid ester of a cyclic alcohol.

5. 2. A transformer oil consisting essentially of a light mineral oil of the transformer oil type and a small proportion, less than about 0.5%, sufficient to inhibit oxidation of said transformer oil, of di-cyclo-hexyl tartrate.

10. 3. A transformer oil consisting essentially of a light mineral oil of the transformer oil type and a small proportion, less than about 0.5%, of a tartaric acid ester of a saturated cyclic alcohol.

15. 4. A transformer oil according to claim 3 substantially free from corrosive soaps.

EARL AMOTT.

### Certificate of Correction

Patent No. 2,397,332.

March 26, 1946.

EARL AMOTT

It is hereby certified that error appears in the printed specification of the above numbered patent requiring correction as follows: Page 2, first column, line 1, beginning with the words "for color" strike out all to and including "ester, the" in line 3, and insert the same in line 6 after "tests"; and that the said Letters Patent should be read with this correction therein that the same may conform to the record of the case in the Patent Office.

Signed and sealed this 10th day of September, A. D. 1946.

[SEAL]

LESLIE FRAZER,  
*First Assistant Commissioner of Patents.*